# EUROPEAN PATENT SPECIFICATION

(11) **EP 0 027 716 B1**
(45) Date of publication and mention of the grant of the patent: **05.03.1986**
(21) Application number: 80303637.5
(22) Date of filing: 15.10.1980
(51) Int. Cl.: D21F 1/00, D03D 1/00

(54) **Dryer felt fabric**
Trockenfilzgewebe
Feutre de séchage tissé

(30) Priority: 17.10.1979 US 85883
(43) Date of publication of application: 29.04.1981
(73) Proprietor: ALBANY INTERNATIONAL CORP., Menards, New York 12201 (US)
(72) Inventor: Josef, Michael J., Clifton Park New York 10265 (US); Romanski, Eric R., Delmar New York 12054 (US)
(74) Representative: Bardo, Julian Eason

## Description

The invention relates to paper machine clothing and more particularly relates to fabrics useful as dryer felts, and their use.

The art is replete with descriptions of dryer felts and dryer felt fabrics. In spite of the wide variety of materials available, the ideal dryer fabric is yet to be found.

In recent years, dryer fabrics have been developed which are constructed partially or entirely from monofilaments. However, such fabrics have not been entirely satisfactory when employed to fashion dryer felts. The monofilaments are subject to abrasion and moist heat hydrolysis. In the prior art constructions the load bearing machine direction monofilament yarns may be rapidly degraded under some conditions of use so that the life of the dryer felt is shortened.

It has also been proposed to use fabrics constructed from monofilaments in the forming sections of paper-making machines. For example, FR-A-2342368 describes a forming wire which is constructed entirely from monofilaments. The wire is a so-called double-layer fabric consisting of two layers of cross-machine direction yarns interwoven by a plurality of machine direction yarns. One layer of cross-machine direction yarns is disposed towards one side of the fabric, providing a fabric first periphery and, likewise, the second layer is disposed towards the other side of the fabric, providing a fabric second periphery.

Double-layer fabrics of this type provide forming wires of greater stability than single-layer fabrics, and do, accordingly, offer a measure of improvement in the forming section of the paper making machine. However, the forming wire is intended to permit the free drainage of extremely large quantities of water from fibres which are being formed into a paper sheet and the required characteristics of the wire differ from those of a dryer felt which is intended to convey the formed paper web around a plurality of heated rollers so that the water remaining in the web is removed by evaporation. The search for an improved dryer felt fabric has, accordingly, continued despite developments in the production of forming wire fabrics.

The present invention provides a paper making machine including a fabric comprising:
a first sinuous layer of cross-machine direction yarns, providing a fabric first periphery of peaks and valley.floors wherein a plurality of peaks are in a first outside plane and a plurality of valley floors are in a first inside plane; a
a second sinuous layer of cross-machine direction yarns, providing a fabric second periphery of peaks and valley floors wherein a plurality of peaks are in a second outside plane and a plurality of valley floors are in a second inside plane; and
a plurality of monofilament machine direction yarns positioned between the first and second outside planes and interweaving the cross-machine direction yarns of the first and second layers,
characterized in that the machine direction yarns interweave the cross-machine direction yarns of the first layer at points within and spaced from the outside and inside planes of the first layer; in that the fabric is provided in the dryer section of the machine for use as a paper making machine dryer felt, and in that the outside plane of the first layer defines a paper contacting plane.

Preferably, the machine direction yarn interweave the cross-machine direction yarns of the second layer at points within and spaced from the outside and inside planes of the second layer.

With the structured fabric employed as a dryer felt in the machine of the present invention, the cross-machine direction yarns support the paper sheet being dried. The monofilament machine direction yarns are thus protected from direct contact with degradative elements. The overall operating life of the dryer felt is significantly increased over felts where the monofilament machine direction yarns are in contact with the paper sheet being dried.

By way of example, an illustrative embodiment of the invention will now be described with reference to the accompanying drawings, of which:
Figure 1 is a cross-sectional, side elevation of a portion of a preferred embodiment fabric of the invention.
Figure 2 is a schematic view of a portion of a drying section in a paper making machine.

Figure 1 is an enlarged, cross-sectional, side elevation of a portion of a fabric 10 embodying the invention. The fabric 10 comprises a first sinuous layer 12 of monofilament cross-machine direction yarns 14. The layer 12 forms a periphery of fabric 10 which in side profile shows peaks 16 and valley floors 18. A plurality of at least two peaks 16 in layer 12 are in a single plane forming an outer periphery of fabric 10. Preferably at least about 50 percent, most preferably all or substantially all of the peaks 16 are in the aforesaid plane. Valley floors 18 are in a separate plane inside of the plane formed by the peaks 16.

A second sinuous layer 20 of monofilamentcross-machine direction yarns 14'forms another periphery of the fabric 10 which also appears, in side profile, as peaks 16' and valley floors 18'. A plurality of at least two of the peaks 16' are in a single plane forming the outer periphery (preferably at least about 50 percent, most preferably all of the peaks 16' are in the periphery). Valley floors 18' are in a separate, single plane inside of the plane formed by peaks 16'.

A plurality of monofilament machine direction yarns 22 are positioned between the outer fabric periphery formed by the outside planes, formed by the peaks 16 and the peaks 16' and interweave with the cross-machine direction yarns 14, 14' at points between the respective planes of peaks 16, valley floors 18 and peaks 16', valley floors 18'. Thus, as shown in Figure 1, the knuckles of load bearing machine direction yarns 22 are below the peaks 16, 16' at the point where they interweave with the cross-machine direction yarns 14,14' and do not come into direct contact with the sheet 24 of paper carried on fabric 10, when fabric 10 is employed as a dryer fabric on a paper making machine. The sheet 24 is supported on the peaks 16 of the cross-machine direction yarn 14. On the side of fabric 10 facing away from the carried sheet, the machine direction yarns 22 are also protected by the outwardly projecting peaks 16' from contact with elements of the paper making machine which might hasten abrasion or other degradation of the important load bearing machine direction yarns. However, it will be appreciated that the greatest degradation of yarns in a dryer fabric occurs in those monofilament yarns in contact with sheet 24. Thus, it is not critical that yarns 22 be protected by peaks 16' on the side of the fabric facing away from the carried sheet 24 although such is obviously preferred. Within the scope of the invention are fabrics where the yarns 22 are on the outer periphery of layer 20 where they pass through layer 20.

In the embodiment fabric 10 the machine direction yarns 22 within layer 12 are paired with the yarns 22 within layer 20 and the yarns within the pairs are slightly offset from each other in regard to vertical alignment, as they knuckle over the cross-machine direction yarns 14, 14'. There are, in the weaving pattern, 4 sets of machine direction yarn 22 pairs. One pair interweaves with every fourth of cross-machine direction yarns 14, 14' and then the pattern repeats. Preferably, the machine direction yarns pass over at least one cross-machine direction yarn, under at least one following cross-machine direction yarn and over at least one further following cross-machine direction yarn of the upper cross-machine direction layer before running down to interconnect the lower cross-machine direction layer with the upper cross-machine direction layer, the machine yarns and cross-machine direction yarns being thus interconnected in a repeat pattern. Of course the weave will be such that the relationship of the machine direction yarns and the upper layer of cross-machine direction yarns will be such that the plane of the upper surfaces of the portions of the cross-machine direction yarns of the upper layer over which the machine direction yarns pass is relatively elevated in a direction away from the plane of the upper surface of the fabric; and the plane of the exposed upper surfaces of the portions of the machine direction yarns in the upper layer under which the cross-machine direction yarns pass is relatively depressed in the opposite direction, whereby the differences in elevation between the exposed upper surface portions of the machine directly yarns are protected from contact with paper sheet which contacts the surface of the cross-machine direction yarns in the upper layer.

The yarns 14,14' and 22 may be monofilaments of any synthetic polymeric resin. The yarns 14 and 14' may also be multifilament yarns. Representative of such multi- and monofilaments are yarns of polyester, polyamide, polyolefin, polyaramid, polyimide and the like. Generally such yarns having diameters of from 10 to 40 mils are advantageously employed in the fabrics of the invention.

Following the weaving of the fabrics of the invention, they are heat set to stabilize the fabric and to draw the yarns into their desired relative positions. The machine direction yarns 22 are drawn inwardly of the outer surfaces of the fabric 10 and this pressure "crimps" the yarns 18, 18' so that the peaks 16, 16' are displaced to the outside plane of the fabric as previously described. The degree of heat-setting required to achieve the desired structure of the fabric 10 will of course vary depending on the nature of the yarns 14, 14' and 22. However, optimum times, temperatures and tensions placed on the fabric during heat-setting can be determined by those skilled in the art, employing trial and error technique for the different yarn materials. In general, heat-setting may be carried out at temperatures of from about 150°F. to 375°Fforfrom 15 to 60 minutes. The fabrics of the invention may be woven flat and the ends joined by conventional seaming methods, known to those skilled in the art. The seamed belts so made are readily employed as dryer felts in the dryer section 30 of a paper making machine as shown in Figure 2. As shown in Figure 2, the paper sheet 24 is held against the steam cylinders 32 by the endless belt 34 of fabric 10 during passage of sheet 24 through dryer section 30.

The following example sets forth the best mode contemplated by the inventors of making and using the invention but is not to be considered as limiting.

### Example 1

A fabric is prepared in a duplex weave of 0.020" diameter polyester monofilament (24 per inch) machine direction yarns and 0.020" diameter polyamide monofilament machine direction yarns (24 per inch) for a total of 48 machine direction yarns per inch interwoven with 0.020" diameter polyester monofilament (48 per inch; 24 top and 24 bottom) filling or cross-machine direction yarns. After heat setting, a fabric is obtained having only cross-machine direction yarns in the outer plane of the fabric. A representative portion of the fabric prepared is subjected to physical testing. The physical properties found are shown in Table I, below.

### Example 2

This is not an example of the invention, but is made for comparison purposes. A fabric is woven in a duplex weave (4 warps and 8 pick repeat) with machine and cross-machine direction yarns as follows:
machine direction-.020" diameter polyester monofilament at 24 per inch.
.020" diameter polyamide monofilament at 24 per inch.
"laid out in a two and two arrangement"
filling-.020" diameter polyester monofilament at 25 per inch. 12.5 top and 12.5 bottom.

After heat-setting, a fabric is obtained wherein the machine direction yarns are in the outer plane of the fabric where they knuckle over the cross-machine direction yarns.

A representative portion of the fabric is tested for its physical properties. The test results are given in Table I, below.

Taber abrasion test

Those skilled in the art will appreciate that many modifications of the preferred embodiments described above may be made without departing from the scope of the invention as defined by the appended claims. For example, the fabric of the invention may be woven to include various stuffer picks, to obtain fabrics of different permeabilities as will be appreciated by those skilled in the art.

## Claims

1. A paper making machine including a fabric (10) comprising:
a first sinuous layer (12) of cross-machine direction yarns (14), providing a fabric first periphery of peaks (16) and valley floors (18) wherein a plurality of peaks (16) are in a first outside plane and a plurality of valley floors (18) are in a first inside plane;
a second sinuous layer (20) of cross-machine direction yarns (14'), providing a fabric second periphery of peaks (16') and valley floors (18') wherein a plurality of peaks (16') are in a second outside plane and a plurality of valley floors (18') are in a second inside plane; and
a plurality of monofilament machine direction yarns (22) positioned between the first and second outside planes and interweaving the cross-machine direction yarns (14,14') of the first and second layers,
characterized in that the machine direction yarns (22) interweave the cross-machine direction yarns (14) of the first layer (12) at points within and spaced from the outside and inside planes of the first layer; in that the fabric (10) is provided in the dryer section (30) of the machine for use as a paper making machine dryer felt, and in that the outside plane of the first layer defines a paper contacting plane.

2. A paper making machine according to claim 1 further characterized in that the machine direction yarns (22) interweave the cross-machine direction yarns (14') of the second layer (20) at points within and spaced from the outside and inside planes of the second layer.

3. A paper making machine according to claim 2 further characterized in that at least 50 per cent of the peaks (16) of the first layer (12) are in the first outside plane.

4. A paper making machine according to any preceding claim further characterized in that at least 50 per cent of the peaks (16') of the second layer (20) are in the second outside plane.

5. A paper making machine according to any preceding claim further characterized in that all the peaks (16) of the first layer (12) are in the first outside plane, all the valley floors (18) of the first layer (12) are in the first inside plane, all the peaks (16') of the second layer (20) are in the second outside plane and all the valley floors (12') of the second layer (20) are in the second inside plane.

6. A paper making machine according to any preceding claim further characterized in that the cross-machine direction yarns (14, 14') are monofilaments.

7. A paper making machine according to any of claims 1 to 5 further characterized in that the cross-machine direction yarns (14, 14') are multifilament yarns.

8. A method of making paper, involving the use of a paper making machine as claimed in any one of claims 1 to 7.

## Patentansprüche

1. Papierherstellungsmaschine einschließlich eines Tuchs (10), umfassend:
eine erste sinusförmige Schicht (12) von quer zur Maschinenrichtung verlaufenden Fäden (14), die eine erste Tuchaußenfläche von Kuppen (16) und Talböden (18) liefern, wobei sich eine Vielzahl von Kuppen (16) in einer ersten außenseitigen Ebene und eine Vielzahl von Talböden (18) in einer ersten innenseitigen Ebene befinden;
eine zweite sinusförmige Schicht (12) von quer zur Maschinenrichtung verlaufenden Fäden (14'), die eine zweite Tuchaußenfläche von Kuppen (16') und Talböden (18') liefern, wobei sich eine Vielzahl von Kuppen (16') in einer zweiten außenseitigen Ebene und eine Vielzahl von Talböden (18') in einer zweiten innenseitigen Ebene befinden; und
eine Vielzahl von in Maschinenrichtung verlaufenden Monofilamentfäden (22) zwischen der ersten und zweiten außenseitigen Ebene angeordnet und die quer zur Maschinenrichtung verlaufenden Fäden (14,14') der ersten und zweiten Schicht verflechtend,
dadurch gekennzeichnet, daß die in Maschinenrichtung verlaufenden Fäden (22) die quer zur Maschinenrichtung verlaufenden Fäden (14) der ersten Schicht (12) an Stellen innerhalb und mit Abstand von den außen- und innenseitigen Ebenen der ersten Schicht durchflechten; daß das Tuch (10) in der Trockenpartie (30) der Maschine zur Verwendung als ein Papierherstellungsmaschinentrockenfilz vorgesehen ist; und daß die außenseitige Ebene der ersten Schicht eine Papierberührungsebene definiert.

2. Papierherstellungsmaschine nach Anspruch 1, weiter dadurch gekennzeichnet, daß die in Maschinenrichtung verlaufenden Fäden (22) die quer zur Maschinenrichtung verlaufenden Fäden (14') der zweiten Schicht (20) an Stellen innerhalb und mit Abstand zu den außen- und innenseitigen Ebenen der zweiten Schicht durchflechten.

3. Papierherstellungsmaschine nach Anspruch 2, weiter dadurch gekennzeichnet, daß wenigstens 50 Prozent der Kuppen (16) der ersten Schict (12) sich in der ersten außenseitigen Ebene befinden.

4. Papierherstellungsmaschine nach irgendeinem vorhergehenden Anspruch, weiter dadurch gekennzeichnet, daß wenigstens 50 Prozent der Kuppen (16') der zweiten Schicht (20) sich in der zweiten außenseitigen Ebene befinden.

5. Papierherstellungsmaschine nach irgendeinem vorhergehenden Anspruch, weiter dadurch gekennzeichnet, daß alle Kuppen (16) der ersten Schicht (12) in der ersten außenseitigen Ebene, alle Talböden (18) der ersten Schicht (12) in der ersten innenseitigen Ebene, alle Kuppen (16') der zweiten Schicht (20) in der zweiten außenseitigen Ebene und alle Talböden (12') der zweiten Schicht (20) in der zweiten innenseitigen Ebene liegen.

6. Papierherstellungsmaschine nach irgendeinem vorhergehenden Anspruch, weiter dadurch gekennzeichnet, daß die quer zur Mschinenrichtung verlaufenden Fäden (14, 14') Monofilamente sind.

7. Papierherstellungsmaschine nach irgendeinem der Ansprüche 1 bis 5, weiter dadurch gekennzeichnet, daß die quer zur Maschinenrichtung verlaufenden Fäden (14, 14') Multifilamente sind.

8. Verfahren zur Papierherstellung, umfassend die Verwendung einer Papierherstellungsmaschine wie in irgendeinem der Ansprüche 1 bis 7 beansprucht.

## Revendications

1. Une machine de fabrication de papier comportant un tissu (10) comprenant:
- une première couche sinueuse (12) de fils (14) orientés dans la direction transversale de machine, en formant une première périphérie de tissu comportant des sommets (16) et des fonds de vallées (18) où une pluralité de sommets (16) sont situés dans un premier plan extérieur et où une pluralité de fonds de vallées (18) sont situés dans un premier plan intérieur;
- une seconde couche sinueuse (20) de fils (14') orientés dans la direction transversale de machine, en formant une seconde périphérie de tissu comportant des sommets (16') et des fonds de vallées (18') et où une pluralité de sommets (16') sont situés dans un second plan extérieur et une pluralité de fonds de vallées (18') sont situés dans un second plan intérieur; et
- une pluralité de fils (22) à monofilaments orientés dans la direction de machine, positionnés entre les premier et second plans extérieurs et entrelacés par tissage avec les fils (14, 14') orientés dans la direction transversale de machine des première et seconde couches,
caractérisée en ce que les fils (22) orientés dans la direction de machine sont entrelacés par tissage avec les fils (14) orientés dans la direction transversale de machine de la première couche (12) en des points situés à l'intérieur et espacés des plans extérieur et intérieur de la première couche; en ce que le tissu (10) est disposé dans la section de séchage (30) de la machine pour être utilisé comme un feutre sécheur de machine de fabrication de papier, et en ce que le plan extérieur de la première couche définit un plan de contact avec le papier.

2. Une machine de fabrication de papier selon la revendication 1, caractérisée en outre en ce que les fils (22) orientés dans la direction de machine sont entrelacées par tissage avec les fils (14') orientés dans la direction transversale de machine de la seconde couche (20) en des points situés à l'intérieur et espacés des plans extérieur et intéieur de la seconde couche.

3. Une machine de fabrication de papier selon la revendication 2, caractérisée en outre en ce qu'au moins 50% des sommets (16) de la première couche (12) sont situés dans le premier plan extérieur.

4. Une machine de fabrication de papier selon une quelconque des revendications précédentes, caractérisée en outre en ce qu'au moins 50% des sommets (16') de la seconde couche (20) sont situés dans le second plan extérieur.

5.. Une machine de fabrication de papier selon une quelconque des revendications précédentes, caractérisée en outre en ce que tous les sommets (16) de la première couche (12) sont situés dans le premier plan extérieur, tous les fonds de vallées (18) de la première couche (12) sont situés dans le premier plan intérieur, tous les sommets (16') de la seconde couche (20) sont situés dans le second plan extérieur et tous les fonds de vallées (12') de la second couche (20) sont situés dans le second plan intérieur.

6. Une machine de fabrication de papier selon une quelconque des revendications précédentes, caractérisée en outre en ce que les fils (14,14') orientés dans la direction transversale de machine sont des monofilaments.

7. Une machine de fabrication de papier selon une quelconque des revendications 1 à 5, caractérisée en outre en ce que les fils (14, 14') orientés dans la direction transversale de machine sont des fils à multifilaments.

8. Un procédé de fabrication de papier, consistant à utiliser une machine de fabrication de papier telle que revendiquée dans une quelconque des revendications 1 à 7.
